

Oct. 17, 1933.

L. E. CALKINS

1,931,018

MANUFACTURE OF CEMENT PRODUCTS

Filed June 27, 1930

Fig. 1,



Fig. 2,



Fig. 3,



Fig. 4



INVENTOR  
Lloyd E. Calkins  
BY  
*Peeters & Cetera, Inc.*  
ATTORNEY

## UNITED STATES PATENT OFFICE

1,931,018

## MANUFACTURE OF CEMENT PRODUCTS

Lloyd E. Calkins, Joliet, Ill., assignor to The  
Rubberoid Co., Bound Brook, N. J., a corpora-  
tion of New Jersey

Application June 27, 1930. Serial No. 464,280

6 Claims. (Cl. 25—155)

This invention relates to the manufacture of cement products and more particularly to the production of asbestos-cement shingles. According to a method now commonly used, such shingles are made by building up layers of the wet mixture of hydraulic cement and fibres on a rotary drum to form a composite sheet of desired thickness. The sheet is stripped from the drum and cut into shingles of the desired size and shape. The shingles are then assembled in a stack with metal plates placed on the top and bottom of the stack and inserted between each succeeding shingle. The stack is then subjected to heavy pressure in a suitable apparatus such as a hydraulic press.

The object of this invention is to facilitate the production of the shingles and lessen the cost of manufacture by reducing the number of metal plates required in the pressing operation.

I have found that a superior product may be produced by dispensing with certain metal plates and inserting a relatively thin flexible membrane between the faces of alternate shingles of the stack. Where metal plates are used throughout, the shingles, when pressed, have a flat smooth surface, but by use of a flexible membrane between alternate shingles, I am able to produce a shingle having an uneven rough surface of pleasing appearance.

In the accompanying drawing,

Figure 1 is a diagrammatic view of a press, showing a stack of shingles positioned therein,

Fig. 2 is a sectional view of a part of the assembled stack,

Fig. 3 is a face view of one of the shingles, and, Fig. 4 is a sectional elevation thereof.

According to the preferred method of carrying out my invention, I take the asbestos-cement shingles 10 and lay them face to face with a relatively thin sheet of membranous material 11 in between the opposed faces of the shingles. The sheet of membranous material may consist of waxed paper or any other material that will not adhere to the shingle. The usual steel plates 13 are then placed on the top and bottom of each pair of shingles and this procedure is repeated until a stack of the desired height is formed.

The stack so assembled is then placed in a suitable press 14, such as a hydraulic press, and subjected to heavy pressure.

As the asbestos-cement composition of which the shingles is formed is not of uniform density or hardness throughout, the pressing operation

will result in the production of shingles having an irregular wavy surface. By using a membrane 11 having a characteristic texture, the texture of the membrane may also be impressed in the faces of the opposed shingles.

While I prefer to employ the invention in the manner stated, it will be obvious that similar membranous sheets may be used on the top and bottom of each pair of shingles instead of placing metal plates thereon. In this case both the back and the face of the shingle will have a roughened appearance.

What I claim is:

1. A method of pressing relatively flat articles composed of hydraulic cement and fibers which consists in arranging the articles face to face with a flexible membrane between their opposed faces, and subjecting the articles so arranged to pressure.

2. A method of pressing relatively flat articles composed of hydraulic cement and fibers which consists in arranging the articles face to face with a flexible membrane between their opposed faces and metal plates on the top and bottom of the pair of articles, and subjecting the articles so arranged to pressure.

3. A method of pressing relatively flat articles composed of hydraulic cement and fibers which consists in arranging the articles in a stack with relatively thin sheets of pliable non-metallic material of a character not to adhere to the cement inserted between alternate articles, and subjecting the stack so formed to pressure.

4. A method of pressing asbestos-cement shingles which consists in taking a pair of shingles and laying them one above the other with a sheet of membranous material in between, forming a stack of a plurality of such pairs, and subjecting the stack to pressure.

5. A method of pressing asbestos-cement shingles which consists in forming a stack composed of shingles arranged face to face with a flexible membrane between their opposed faces and with metal plates on the top and bottom of each pair, and subjecting the stack to pressure.

6. A method of pressing asbestos-cement shingles which consists in forming a stack composed of shingles arranged face to face with a sheet of pliable waxed paper between their opposed faces and with metal plates on the top and bottom of each pair, and subjecting the stack to pressure.

LLOYD E. CALKINS.